

May 22, 1923.

1,456,370

W. H. DRAKE ET AL

PROCESS OF MAKING WATERPROOF RIGID ARTICLES FROM PULP

Filed Feb. 2, 1920



Fig. 1.



Fig. 2.

Inventors.

Walter H. Drake  
James J. Drake

By Bradford Morris Bissell  
Attorney

## UNITED STATES PATENT OFFICE.

WALTER HENRY DRAKE AND JAMES JOSEPH DRAKE, OF CLEVELAND, OHIO.

## PROCESS OF MAKING WATERPROOF RIGID ARTICLES FROM PULP.

Application filed February 2, 1920. Serial No. 355,827.

*To all whom it may concern:*

Be it known that we, WALTER HENRY DRAKE and JAMES JOSEPH DRAKE, citizens of the United States, residing at Cleveland, 5 in the county of Cuyahoga and State of Ohio, have invented certain new and useful Improvements in Processes of Making Waterproof Rigid Articles from Pulp, of which the following is a specification.

10 This invention relates to the process of making water proof rigid articles from pulp and has for an object to produce such articles by depositing upon the walls of a foraminous mold, pulp, the fibers of which are 15 treated with a binder, which when heated, fuse and form an intimate mass, and when cooled, become rigid and impervious.

The drawings illustrate conventionally an apparatus in which the process may be carried out, it being understood that such drawing is shown only for the purpose of illustrating the steps of the process and in no way effect the process as such. Such drawings show at Figure 1, a vertical diametrical sectional view with the mold closed and Figure 2, shows a vertical diametrical sectional view with the mold open to discharge the completed article.

In the carrying out of the present process, 30 the pulp is prepared in any usual and ordinary manner, as it might be prepared for paper making or the like and at any step of the process, but preferably in the beater, the pulp is treated with a material which later 35 will produce the water proofing and rigidifying binder. The material so added is the usual and ordinary sizing material consisting in first emulsifying the pulp by the addition thereto of rosin soap, known as paper makers' soap, and after the formation of 40 such emulsion, adding thereto alum, which reacts with the emulsified rosin to produce an aluminum resinate, which is precipitated as a coating upon each and every individual 45 fiber of the pulp. The pulp so treated with the aluminum resinate is conducted to the receptacle 10, as shown in the drawings. From the receptacle 10, a conduit 12 depends, controlled by a valve 14, and with 50 a valved pipe 15 introduced below the valve 14. To the conduit member 12 the mold

sections 16 and 17 are hinged, so that they may be closed together as shown at Figure 1 in position to receive the inflowing pulp, or may be separated as shown at Figure 2, 55 for the purpose of discharging the completed article. As shown in the drawing the shape of the foraminous mold indicates the production of a milk bottle, but it is to be understood that such form, shape and proportion are in no way limiting upon the invention and that the invention includes the production of containers of other shapes, sizes and proportions and articles other than containers. 60

From the conduit 12, a duct 18, depends preferably coinciding with the axis of the mold and extending nearly to the bottom thereof. A telescoping section 19 is preferably formed upon the end of the duct 18, 70 for the purpose of regulating the point of discharge of the pulp within the mold. The discharge of the pulp in this manner and the deposition of the pulp upon the walls of the foraminous mold, is not novel in the 75 present application, being the subject matter of Patent No. 1,305,203, issued May 27, 1919.

The pulp carrying the aluminum resinate is discharged into the mold and by reason 80 of the position of the duct and the force of the inflow of pulp, the pulp is moved upwardly along the walls of the mold and deposited in a uniform layer upon such walls. When a sufficient amount of the pulp has 85 been deposited to produce the desired thickness of article, the valve 14 is closed to cut off further inflow. Heated air is now admitted through the pipe 15 into the mold, expelling the remainder of the fluid carriage. 90 The air, or if desired, super-heated steam, so employed, is of such temperature as to fuse or melt the aluminum resinate carried by the fibers. The exact temperature of melting or fusing of this aluminum resinate 95 is not known at the present time, but is probably somewhere about 400 degrees F. Aluminum resinate is rigid at a temperature well above the temperature of boiling water, after passing which point it becomes soft- 100 ened and plastic and when the temperature has been raised to a sufficient degree, becomes

fluid. The heat necessary to completely melt or fuse the aluminum resinate, quickly dries the moisture from the pulp, so that it performs the double function of drying the article and fusing the aluminum resinate. It appears that the forcing of the heated air through the pulp does not tend to displace the aluminum resinate coating the individual fibers, but only melts such coating to such an extent that as soon as the heated air is interrupted by closing the valve in the pipe 15, the contiguous fibers adhere by the aluminum resinate becoming substantially a homogeneous mass, rigidifying with the drop of temperature. The use of aluminum resinate as a sizing for paper has never contemplated the fusing thereof, as such fusing and subsequent cooling renders the article rigid which is a condition undesired 20 for paper and inoperative for water proofing for the reason that bending and folding fractures the water proofing substance. For an article wherein rigidity is a desideratum, the fusing and rigidifying of the binder, adds not only the desired water proofing, but also greatly to the rigidity of the article. Taking a container as an example, the aluminum resinate remains rigid well above the temperature of boiling water, so that a container 25 water proofed with this material, is impervious, not only to cold water, but also to boiling water.

Furthermore, the high temperature to which the article is subjected for the purpose 30 of fusing the aluminum resinate, completely antisepticizes the material, so that the article discharged from the mold is not only completely water proofed, but is rigid and aseptic. 40 While alum has been specified as the reagent for acting upon the resinous emulsion, it is undoubtedly true that other reagents may be similarly employed in which case the precipitate would naturally not be aluminum resinate, the exact formula depending upon the reagent employed and where aluminum resinate has been mentioned in this specification, or the claims, it is to be understood that any equivalent resinate is comprehended within the term.

While the drawing would indicate that the intent of this invention is the making of hollow articles that may be made in a separable mold, it is to be understood that 50 it is not so limited and that it comprehends the making of any article of whatever shape as for instance composite board or the article of commerce ordinarily known as "wall board" or any article for any purpose where a rigid waterproof pulp article would be desirable.

We claim:—

1. The process of water-proofing an article composed of fiber, consisting in coating

the fibers with aluminum resinate, depositing the coated fibers in the required form, and forcing through the fibrous mass a fluid heated to the temperature of melting of the aluminum resinate.

2. The process of water-proofing an article composed of pulp, consisting in treating the pulp with materials to precipitate aluminum resinate upon the fibers, depositing the coated fibers upon a surface having the required contour, and subjecting the fibrous deposit to a heat sufficient to melt and fuse the aluminum resinate while still in contact with the contoured surface.

3. The process of water-proofing and rigidifying an article composed of pulp, consisting in depositing the fibers of the pulp upon a surface having the required contour and depositing therewith a binder material adapted to be fused and melted by the application of heat thereto and to become rigid at a temperature above the temperature of boiling water.

4. The process of water-proofing an article composed of pulp, consisting in depositing the fibers of pulp upon a contoured surface commingled with a resinous material capable of being fused and melted by the application of heat thereto and to become rigid at a temperature above the temperature of boiling water, and applying a sufficient degree of heat to the pulp while in contact with the contoured surface to fuse and melt the binder.

5. The process of water-proofing an article composed of pulp, consisting in employing a foraminous mold introducing the pulp under pressure to the foraminous mold, to deposit the pulp fibers and discharge the carriage, commingling with the pulp fibers so deposited a binding material capable of melting by the application of heat and to become rigid at a temperature above the temperature of boiling water and subjecting the article to heat while contained within the mold.

6. The process of water-proofing an article composed of pulp, consisting in commingling with the pulp an aluminum resinate, depositing the commingled pulp fibers and aluminum resinate upon a foraminous surface, and forcing through the pulp deposit and foraminous surface, a fluid heated to a temperature to melt and fuse the aluminum resinate.

7. The process of waterproofing an article composed of pulp consisting in commingling with the pulp fibers a resinous binder, depositing the commingled materials upon a contouring surface, removing the aqueous carriage and fusing the binder while yet in contact with the contouring surface.

8. The process of waterproofing an article composed of pulp consisting in emulsify-

ing the pulp with a resinous saponifier, precipitating the resins on to the pulp fibers in the form of aluminum resinate by the addition of alum to the emulsion, contouring

5 the pulp and driving off the carriage by forcing therethrough anhydrous fluid at a temperature to fuse the aluminum resinate.

In witness whereof, we have hereunto set our hands and seals at Cleveland, Cuyahoga County Ohio this 31st day of January, A. 10 D., nineteen hundred and twenty.

WALTER HENRY DRAKE. [ L. S. ]  
JAMES JOSEPH DRAKE. [ L. S. ]